# EUROPEAN PATENT SPECIFICATION

(11) **EP 2 281 924 B1**
(45) Date of publication and mention of the grant of the patent: **16.04.2014**
(21) Application number: 10251383.5
(22) Date of filing: 03.08.2010
(51) Int. Cl.: C23C 28/00, C23C 28/04

(54) **Structually diverse thermal barrier coatings**
Strukturelle unterschiedliche Wärmedämmbeschichtungen
Revêtements de barrière thermique structurellement différents

(30) Priority: 04.08.2009 US 534945
(43) Date of publication of application: 09.02.2011
(73) Proprietor: United Technologies Corporation, Hartford, CT 06101 (US)
(72) Inventor: Tryon, Brian S., Glastonbury, CT 06033 (US); Schlichtung, Kevin W., South Glastonbury, CT 06073 (US); Freling, Melvin, West Hartford, CT 06117 (US); Litton, David A., West Hartford, CT 06107 (US)
(74) Representative: Leckey, David Herbert

(56) References cited:
- EP-A1- 0 605 196
- EP-A1- 1 085 109
- EP-A1- 1 400 611
- EP-A1- 1 536 039
- EP-A1- 1 591 550
- EP-A1- 1 790 754
- EP-A1- 1 806 432
- EP-A1- 1 821 333
- EP-A1- 1 900 708
- EP-A2- 1 550 642
- EP-B1- 0 193 429
- WO-A1-2004/029330
- WO-A2-2004/076704
- US-A- 5 876 860
- US-A- 6 054 184
- US-A1- 2002 110 698
- US-A1- 2003 138 658
- US-B1- 6 306 517
- MA W ET AL: "Yb2O3 and Gd2O3 doped strontium zirconate for thermal barrier coatings", JOURNAL OF THE EUROPEAN CERAMIC SOCIETY, ELSEVIER SCIENCE PUBLISHERS, BARKING, ESSEX, GB, vol. 28, no. 16, 1 December 2008 (2008-12-01), pages 3071-3081, XP025432453, ISSN: 0955-2219, DOI: 10.1016/J.JEURCERAMSOC.2008.05.013 [retrieved on 2008-06-30]
- HONG-SONG Z ET AL: "Preparation and thermophysical properties of (Sm0.5La0.5)2Zr2O7 and (Sm0.5La0.5)2 (Zr0.8Ce0.2)2O7 ceramics for thermal barrier coatings", JOURNAL OF ALLOYS AND COMPOUNDS, ELSEVIER SEQUOIA, LAUSANNE, CH, vol. 475, no. 1-2, 5 May 2009 (2009-05-05) , pages 624-628, XP026035621, ISSN: 0925-8388 [retrieved on 2008-09-18]
- KE P L ET AL: "Study on thermal barrier coatings deposited by detonation gun spraying", SURFACE AND COATINGS TECHNOLOGY, ELSEVIER, AMSTERDAM, NL, vol. 200, no. 7, 21 December 2005 (2005-12-21), pages 2271-2276, XP027608594, ISSN: 0257-8972 [retrieved on 2005-12-21]

## Description

### BACKGROUND

The invention relates to thermal barrier coatings and, more particularly, relates to reduced conductivity thermal barrier coating systems having at least two layers, each layer exhibiting a different microstructure.

Thermal barrier coatings (hereinafter "TBCs") are employed in turbine engines in an effort to shield and protect the structural metallic components from the high temperature conditions present in a combustion environment. EP 1536039 A1 discloses a thermal barrier coating. WO 2004/029330 A discloses a thermal barrier coating having the features of the preamble of claim 1. US 2002/0110698 A1 describes thermal barrier coatings and electron beam, physical vapour deposition for making same. These ceramic coatings effectively lower the substrate metal surface temperature and slow the kinetics of oxidation which degrades the metallic substrate. Reduced conductivity TBCs have provided an even greater benefit to turbine engines than conventional TBCs by allowing higher turbine engine operation temperatures or even further reduced metal substrate temperatures. The microstructure of a TBC is dictated by processing. The microstructure also contributes to the physical properties of the coated article, in particular, the thermal conductivity. When creating thermal barrier coatings, it is desirable to reduce the thermal conductivity of the TBCs as much as possible.

### SUMMARY

In one aspect of the present disclosure, there is provided a coated article as claimed in claim 1.

In one embodiment, the coated article is a turbine engine component.

In another aspect of the present disclosure, there is provided a process for coating an article as claimed in claim 10.

The details of one or more embodiments of the invention are set forth in the accompanying drawings and the description below. Other features, objects, and advantages of the invention will be apparent from the description and drawings, and from the claims.

### BRIEF DESCRIPTION OF THE DRAWINGS

FIG. 1 is a flowchart of an exemplary process for coating an article according to the present disclosure;
FIG. 2 is a representation of an exemplary embodiment of a bi-layered reduced conductivity TBC exhibiting different microstructures and/or morphologies; and
FIG. 3 is a representation of another exemplary embodiment of a multi-layered reduced conductivity TBC exhibiting different microstructures and/or morphologies.

Like reference numbers and designations in the various drawings indicate like elements.

### DETAILED DESCRIPTION

Referring to FIG. 1, an exemplary process for coating an article according to the present disclosure is illustrated. The article to be coated may comprise a turbine engine component to which a reduced thermal conductivity thermal barrier coating system may be applied. The exemplary thermal barrier coating system exhibits a thermal conductivity of no more than about 16 BTU in/hr ft² F (2.31 W/mK). The thermal barrier coating system as described herein increases the surface temperature capability of the coated article. In a first embodiment of the present invention, the thermal conductivity of the thermal barrier coating system may be in the range of 2.0 to 16 BTU in/hr ft² F (0.29 to 2.31 W/mK). In a second embodiment of the present invention, the thermal conductivity of the thermal barrier coating system may be in the range of from 4.0 to 14 BTU in/hr ft² F (0.58 to 2.02 W/mK). In yet another embodiment of the present invention, the thermal conductivity of the thermal barrier coating system may be in the range of from 4.0 to 10 BTU in/hr ft² F (0.58 to 1.44 W/mK).

If desired, an optional bond coat layer may be applied on at least one surface of the article at step 10 prior to the application of the thermal barrier coating system. The bond coat layer may be applied using any suitable technique known in the art. If desired, a thermally grown oxide layer ("TGO") may be formed upon the bond coat layer at step 12 using any suitable technique known in the art. Alternatively, the thermal barrier coating system may be directly applied to, or deposited on, the at least one surface of the article.

A first layer of a thermal barrier coating may be applied upon the at least one surface of the article, or the bond coat layer if present or the thermally grown oxide layer if present, at step 14. A second layer of the thermal barrier coating may be deposited on the first layer at step 16. During the second layer deposition process, an interlayer typically forms between the first and second layers of the thermal barrier coating at step 18. One or more additional layers may be applied upon the second layer at step 20 such that additional interlayer(s) form between each layer subsequently applied at step 22. Each layer of the thermal barrier coating system preferably has a different microstructure. The first layer has a first microstructure, the second layer has a second microstructure, and the interlayer has a microstructure exhibiting a combination of the first and second microstructures.

The application of the bond coat and the first, second and any subsequent layers of the thermal barrier coating system may be achieved using either a vapor deposition process (e.g., physical vapor deposition) or a thermal spray process (e.g., plasma spraying) as known to one of ordinary skill in the art. Whether using a vapor deposition process or a thermal spray process, each layer of the thermal barrier coating system, and the bond coat layer, is applied so that each layer exhibits a different microstructure. The microstructures contemplated herein include, but are not limited to, columnar, amorphous, randomized, and splat-like microstructures. Whether using a vapor deposition process or a thermal spray process, each layer of the thermal barrier coating may be applied using a vacuum-plasma spraying torch apparatus known as the O3CP, commercially available from Sulzer Metco Ltd., of Westbury, New York. The O3CP vacuum-plasma spraying apparatus allows a user to apply a first coating exhibiting a microstructure such as the claimed columnar microstructure, and then adjust the operating parameters of the spraying apparatus to apply a subsequent coating exhibiting a different microstructure. Prior processes required one of ordinary skill in the art to utilize two entirely different spraying apparatus to apply coatings having different microstructures as disclosed herein. In using the O3CP vacuum-plasma spraying apparatus to perform the exemplary process described herein, one recognizes benefits such as reduced time and costs, increased efficiency, and minimized likelihood of contaminating the thermal barrier coating system being applied.

Referring now to FIGS. 2 and 3, these drawings illustrate representations of exemplary coated articles 30, 50 produced according to the exemplary processes described herein. The exemplary thermal barrier coating system having layers exhibiting different microstructures and possessing a reduced thermal conductivity over thermal barrier coating systems having homogeneous microstructures. Each article 30, 50 may comprise a surface 32, 52 having a bond coat layer 34, 54 disposed thereupon. The bond coat may be either a MCrA1Y coating where M is nickel and/or cobalt, an aluminide coating, a platinum aluminide coating, a ceramic based bond coat, or a silica based bond coat. The bond coat layer 34, 54 aids the growth of the TGO 36, 56, which is typically aluminum oxide (Al₂O₃). Specifically, prior to or during application of the exemplary thermal barrier coating system described herein on the bond coat layer, the exposed surface of the bond coat layer 34, 54 can be oxidized to form the TGO 36, 56.

Referring now to FIG. 2, an exemplary thermal barrier coating system 38 may comprise a bi-layer thermal barrier coating. The thermal barrier coating system 38 may comprise a first layer 40 having a first microstructure disposed upon the surface 32 of the article 30, or the bond coat layer 34 or the TGO 36 when present. The coating system 38 may also comprise a second layer 44 having a second microstructure, and an interlayer 42 formed between the first layer 40 and the second layer 44. The interlayer 42 may be formed gradually or abruptly depending upon the transition between the applications of the first layer 40 and the second layer 44. As a result, the interlayer 42 may have a third microstructure possessing a combination of the first and second microstructures, that is, structural elements and variants of the first and second microstructures.

Referring now to FIG. 3, another exemplary thermal barrier coating system 58 may comprise a multi-layered system. Thermal barrier coating system 58 may also comprise the first layer 60, the interlayer 62 and the second layer 64 as described above for thermal barrier coating system 38. In addition, the coating system 58 may comprise a third layer 68 having a fourth microstructure, and another interlayer 66 formed between the second layer 64 and third layer 68. The interlayer 66 may comprise a fifth microstructure. As described above, interlayer 66 may be formed in the same manner such that the fifth microstructure contains structural elements and variants of both the third and fourth microstructures.

Each layer of the thermal barrier coating system may include a ceramic base material and at least one dopant oxide of a metal present in an amount of about 30 wt% to about 70 wt% of the total weight of the layer. Suitable ceramic base materials include any one of the following: a zirconate, a hafnate or a titanate. Suitable dopant oxides of a metal include oxides of any one of the following metals: lanthanum, cerium, praseodymium, neodymium, promethium, samarium, europium, gadolinium, terbium, dysprosium, holmium, erbium, thulium, ytterbium, lutelium, indium, scandium, and yttrium. For example, a representative thermal barrier coating system may comprise yttria stabilized zirconia having from about 1.0 wt% to about 25 wt% yttria of the total weight of the layer and a balance of zirconia, or gadolinia stabilized zirconia having from about 30 wt% to about 70 wt% gadolinia, of the total weight of the layer and a balance of zirconia or both yttria stabilized zirconia and gadolinia stabilized zirconia.

## Claims

1. A coated article, comprising:
an article having at least one surface; and
a thermal barrier coating system (38) disposed upon said at least one surface;
said thermal barrier coating system (38) comprising at least two layers (40,44;60,64,68), wherein:
each of said layers (40,44;60,64,68) has a different microstructure than the other of said layers (40,44;60,64,68);
**characterised in that**:
at least one layer (40,44;60,64,68) of said thermal barrier coating system includes:
a ceramic base material selected from the group consisting of a zirconate, a hafnate and a titanate; and
at least one oxide of a metal present in an amount from about 30 wt% to about 70 wt% of the total weight of said layer, said metal comprising at least one metal selected from the group consisting of lanthanum, cerium, praseodymium, neodymium, promethium, samarium, europium, gadolinium, terbium, dysprosium, holmium, erbium, thulium, ytterbium, lutelium, indium, scandium, and yttrium; and
said thermal barrier coating system (38) exhibits a thermal conductivity of no more than 16 BTU in/hr ft² F (2.31 W/mK), wherein said thermal barrier coating system comprises:
a first layer (40;60) having a first, columnar microstructure;
a second layer (44;64) having a second microstructure selected from the group consisting of amorphous, randomized, and splat-like; and
a first interlayer (42;62) having a third microstructure formed between said first and second layers,
wherein said third microstructure comprises a combination of said first and second microstructures.

2. The coated article of claim 1, wherein said thermal barrier coating system further comprises:
a third layer (68) having a fourth microstructure; and
a second interlayer (66) having a fifth microstructure formed between said second (64) and third (68) layers.

3. The coated article of claim 2, wherein said fourth microstructure has a microstructure selected from the group consisting of columnar, amorphous, randomized, and splat-like;
and optionally wherein said fifth microstructure comprises a combination of said second and fourth microstructures.

4. The coated article of claim 1 wherein:
said article is a turbine engine component;
said thermal barrier coating system (38) wherein said first and second microstructures comprise any one of the following microstructures: columnar, amorphous, randomized, and splat-like; and
said third microstructure comprises a combination of said first and second microstructures.

5. The coated article of claim 4, wherein each layer (40,44;60,64,68) of said thermal barrier coating system (38) comprises yttria stabilized zirconia having from about 1.0 wt% to about 25 wt% yttria of the total weight of said layer and a balance of zirconia or gadolinia stabilized zirconia having from about 5.0 wt% to about 99 wt% gadolinia of the total weight of said layer and a balance of zirconia or both said yttria stabilized zirconia and said gadolinia stabilized zirconia.

6. The coated article of claim 5, wherein said gadolinia stabilized zirconia includes from about 30 wt% to about 70 wt% gadolinia of the total weight of said layer (40,44;60,64,68) and a balance of zirconia.

7. The coated article of claim 4, 5 or 6, further comprising a bond coat layer (34;54) disposed between said at least one surface and said thermal barrier coating system (38);
and optionally further comprising a thermally grown oxide layer (36;56) disposed between said bond coat layer (34;54) and said thermal barrier coating system (38).

8. The coated article of any of claims 4 to 7, wherein said thermal barrier coating further comprises:
a third layer (68) having a fourth microstructure; and
a second interlayer (66) having a fifth microstructure formed between said second (64) and third (68) layers,
wherein said fourth microstructure comprises any one of the following microstructures: columnar, amorphous, randomized, and splat-like, and
wherein said fifth microstructure comprises a combination of said second and fourth microstructures.

9. The coated article of any preceding claim, wherein said thermal conductivity is in the range of from 2.0 to 16 BTU in/hr ft² F (0.29 to 2.31 W/mK).

10. A process for coating an article, comprising:
applying a first layer (40;60) of a thermal barrier coating system (38) having a first, columnar microstructure on at least one surface of an article;
applying upon said first layer (40;60) a second layer (44;64) of said thermal barrier coating system (38) having a second microstructure selected from the group consisting of amorphous, randomized, and splat-like; **characterised by**
forming between said first (40;60) and second (44;64) layers an interlayer (42;62) having a third microstructure comprising a combination of said first and second microstructures; wherein
at least one layer (40,44;60,64,68) of said thermal barrier coating system includes:
a ceramic base material selected from the group consisting of a zirconate, a hafnate and a titanate; and
at least one oxide of a metal present in an amount from about 30 wt% to about 70 wt% of the total weight of said layer, said metal comprising at least one metal selected from the group consisting of lanthanum, cerium, praseodymium, neodymium, promethium, samarium, europium, gadolinium, terbium, dysprosium, holmium, erbium, thulium, ytterbium, lutelium, indium, scandium, and yttrium; and
said thermal barrier coating system (38) exhibits a thermal conductivity of no more than 16 BTU in/hr ft² F (2.31 W/mK).

11. The process of claim 10, further comprising the steps of:
applying a bond coat layer (34;54) upon said at least one surface of said article prior to applying said first layer (40;60); and
forming a thermally grown oxide layer (36;56) upon said bond coat layer (34;54) prior to applying said first layer (40;60); and
wherein, optionally, said steps of applying said first layer (40;60), applying said second layer (44;64) and applying said bond coat layer (34;54) comprise using a vapor deposition process or a thermal spraying process.

## Patentansprüche

1. Beschichteter Gegenstand, aufweisend:
einen Gegenstand mit mindestens einer Oberfläche; und
ein Wärmebarrieren-Beschichtungssystem (38), das auf der mindestens einen Oberfläche angeordnet ist;
wobei das Wärmebarrieren-Beschichtungssystem (38) mindestens zwei Schichten (40, 44; 60, 64, 68) aufweist;
wobei jede der Schichten (40, 44; 60, 64, 68) eine andere Mikrostruktur als die jeweils andere(n) der Schichten (40, 44; 60, 64, 68) aufweist;
**dadurch gekennzeichnet, dass** mindestens eine Schicht (40, 44; 60, 64, 68) des Wärmebarrieren-Beschichtungssystems aufweist:
ein Material auf Keramikbasis, ausgewählt aus der Gruppe bestehend aus einem Zirkonat, einem Hafnat und einem Titanat; und
mindestens ein Oxid eines Metalls, das in einer Menge von etwa 30 Gew.-% bis etwa 70 Gew.-% des Gesamtgewichts der Schicht vorhanden ist, wobei das Metall mindestens ein Metall aufweist, das aus der Gruppe ausgewählt ist, bestehend aus Lanthan, Cer, Praseodym, Neodym, Promethium, Samarium, Europium, Gadolinium, Terbium, Dysprosium, Holmium, Erbium, Thulium, Ytterbium, Lutelium, Indium,
Scandium und Yttrium; und
wobei das Wärmebarrieren-Beschichtungssystem (38) eine Wärmeleitfähigkeit von nicht mehr als 16 BTU in/hr ft² F (2,31 W/mK) aufweist,
wobei das Wärmebarrieren-Beschichtungssystem aufweist:
eine erste Schicht (40; 60) mit einer ersten, säulenförmigen Mikrostruktur;
eine zweite Schicht (44; 64) mit einer zweiten Mikrostruktur,
ausgewählt aus der Gruppe bestehend aus amorph, randomisiert und
klecksartig; und
eine zwischen der ersten und der zweiten Schicht gebildete erste Zwischenschicht (42; 62) mit einer dritten Mikrostruktur,
wobei die dritte Mikrostruktur eine Kombination aus der ersten und
der zweiten Mikrostruktur aufweist.

2. Beschichteter Gegenstand nach Anspruch 1,
wobei das Wärmebarrieren-Beschichtungssystem ferner aufweist:
eine dritte Schicht (68) mit einer vierten Mikrostruktur; und
eine zwischen der zweiten (64) und der dritten (68) Schicht gebildete zweite Zwischenschicht (66) mit einer fünften Mikrostruktur.

3. Beschichteter Gegenstand nach Anspruch 2,
wobei die vierte Mikrostruktur eine Mikrostruktur aufweist, die aus der Gruppe ausgewählt ist, bestehend aus säulenförmig, amorph, randomisiert und klecksartig;
und wobei wahlweise die fünfte Mikrostruktur eine Kombination aus der zweiten und der vierten Mikrostruktur aufweist.

4. Beschichteter Gegenstand nach Anspruch 1,
wobei der Gegenstand eine Turbinenmaschinenkomponente ist; wobei bei dem Wärmebarrieren-Beschichtungssystem (38) die erste und die zweite Mikrostruktur eine beliebige der folgenden Mikrostrukturen aufweisen: säulenförmig, amorph, randomisiert und klecksartig; und
wobei die dritte Mikrostruktur eine Kombination aus der ersten und zweiten Mikrostruktur aufweist.

5. Beschichteter Gegenstand nach Anspruch 4,
wobei jede Schicht (40, 44; 60, 64, 68) des Wärmebarrieren-Beschichtungssystems (38) aufweist: Yttriumoxid-stabilisiertes Zirkonoxid mit etwa 1,0 Gew.-% bis etwa 25 Gew.-% Yttriumoxid des Gesamtgewichts der Schicht, Rest Zirkonoxid- oder Gadoliniumoxidstabilisiertes Zirkonoxid mit etwa 5,0 Gew.-% bis etwa 99 Gew.-% Gadoliniumoxid des Gesamtgewichts der Schicht, Rest Zirkonoxid oder sowohl das Yttriumoxid-stabilisierte Zirkonoxid als auch das Gadoliniumoxid-stabilisierte Zirkonoxid.

6. Beschichteter Gegenstand nach Anspruch 5,
wobei das Gadoliniumoxid-stabilisierte Zirkonoxid etwa 30 Gew.-% bis etwa 70 Gew.% Gadoliniumoxid des Gesamtgewichts der Schicht (40, 44; 60, 64, 68), Rest Zirkonoxid, aufweist.

7. Beschichteter Gegenstand nach Anspruch 4, 5 oder 6,
weiterhin aufweisend eine Haftvermittlungsschicht (34; 54), die zwischen der mindestens einen Oberfläche und dem Wärmebarrieren-Beschichtungssystem (38) angeordnet ist;
und wahlweise weiterhin aufweisend eine thermisch gewachsene Oxidschicht (36; 56), die zwischen der Haftvermittlungsschicht (34; 54) und dem Wärmebarrieren-Beschichtungssystem (38) angeordnet ist.

8. Beschichteter Gegenstand nach einem der Ansprüche 4 bis 7, wobei die Wärmebarrierenbeschichtung ferner aufweist:
eine dritte Schicht (68) mit einer vierten Mikrostruktur; und
eine zwischen der zweiten (64) und dritten (68) Schicht gebildete zweite Zwischenschicht (66) mit einer fünften Mikrostruktur,
wobei die vierte Mikrostruktur eine beliebige der folgenden Mikrostrukturen aufweist: säulenförmig, amorph, randomisiert und klecksartig, und
wobei die fünfte Mikrostruktur eine Kombination aus der zweiten und
der vierten Mikrostruktur aufweist.

9. Beschichteter Gegenstand nach einem der vorhergehenden Ansprüche, wobei die Wärmeleitfähigkeit im Bereich von 2,0 bis 16 BTU in/hr ft² F (0,29 bis 2,31 W/mK) liegt.

10. Verfahren zum Beschichten eines Gegenstandes, mit folgenden Schritten:
Aufbringen einer ersten Schicht (40; 60) eines Wärmebarrieren-Beschichtungssystems (38) mit einer ersten, säulenförmigen Mikrostruktur auf mindestens einer Oberfläche eines Gegenstandes;
auf die erste Schicht (40; 60) erfolgendes Aufbringen einer zweiten Schicht (44; 64) des Wärmebarrieren-Beschichtungssystems (38) mit einer zweiten Mikrostruktur, die aus der Gruppe ausgewählt ist,
bestehend aus amorph, randomisiert und klecksartig;
**gekennzeichnet durch** folgende Schritte:
zwischen der ersten (40; 60) und der zweiten (44; 64) Schicht erfolgendes Bilden einer Zwischenschicht (42; 62) mit einer dritten Mikrostruktur, die eine Kombination aus der ersten und der zweiten Mikrostruktur aufweist;
wobei mindestens eine Schicht (40, 44; 60, 64, 68) des Wärmebarrieren-Beschichtungssystems aufweist:
ein Material auf Keramikbasis, ausgewählt aus der Gruppe bestehend aus einem Zirkonat, einem Hafnat und einem Titanat; und
mindestens ein Oxid eines Metalls, das in einer Menge von etwa 30 Gew.-% bis etwa 70 Gew.-% des Gesamtgewichts der Schicht vorhanden ist, wobei das Metall mindestens ein Metall aufweist, das aus der Gruppe ausgewählt ist, bestehend aus Lanthan, Cer, Praseodym, Neodym, Promethium, Samarium, Europium, Gadolinium, Terbium, Dysprosium, Holmium, Erbium, Thulium, Ytterbium, Lutelium, Indium, Scandium und Yttrium; und
wobei das Wärmebarrieren-Beschichtungssystem (38) eine Wärmeleitfähigkeit von nicht mehr als 16 BTU in/hr ft² F (2,31 W/mK) aufweist.

11. Verfahren nach Anspruch 10,
das weiterhin folgende Schritte aufweist:
Aufbringen einer Haftvermittlungsschicht (34; 54) auf die mindestens eine Oberfläche des Gegenstands vor dem Aufbringen der ersten Schicht (40; 60); und
Bilden einer thermisch gewachsenen Oxidschicht (36; 56) auf der Haftvermittlungsschicht (34; 54) vor dem Aufbringen der ersten Schicht (40; 60); und
wobei wahlweise die Schritte des Aufbringens der ersten Schicht (40; 60), des Aufbringens der zweiten Schicht (44; 64) und des Aufbringen der Haftvermittlungsschicht (34; 54) die Verwendung eines Dampfabscheidungsverfahrens oder eines thermischen Spritzverfahrens beinhalten.

## Revendications

1. Article revêtu, comprenant :
un article ayant au moins une surface ; et
un système de revêtement formant barrière thermique (38) disposé sur ladite au moins une surface ;
ledit système de revêtement formant barrière thermique (38) comprenant au moins deux couches (40, 44 ; 60, 64, 68), dans lesquelles :
chacune desdites couches (40, 44 ; 60, 64, 68) a une microstructure différente des autres desdites couches (40, 44 ; 60, 64, 68) ;
caractérisé en ce qui :
au moins une couche (40, 44 ; 60, 64, 68) dudit système de revêtement formant barrière thermique inclut :
une matière de base en céramique sélectionnée à partir du groupe constitué par un zirconate, un hafnate et un titanate ; et
au moins un oxyde d'un métal présent en une quantité d'environ 30 % en poids à environ 70 % en poids du poids total de ladite couche, ledit métal comprenant au moins un métal sélectionné à partir du groupe constitué par le lanthane, le cérium, le praséodyme, le néodyme, le prométhium, le samarium, l'europium, le gadolinium, le terbium, le dysprosium, l'holmium, l'erbium, le thulium, l'ytterbium, le lutécium, l'indium, le scandium et l'yttrium ; et
ledit système de revêtement formant barrière thermique (38) présente une conductibilité thermique non supérieure à 16 BTU in/hr ft² F (2,31 W/mK), dans lequel ledit système de revêtement formant barrière thermique comprend :
une première couche (40 ; 60) ayant une première microstructure à colonnes ;
une deuxième couche (44 ; 64) ayant une deuxième microstructure sélectionnée à partir du groupe amorphe, aléatoire et semblable à une latte ; et
une première intercouche (42 ; 62) ayant une troisième microstructure formée entre lesdites première et deuxième couches,
dans lequel ladite troisième microstructure comprend une combinaison desdites première et deuxième microstructures.

2. Article revêtu selon la revendication 1, dans lequel ledit système de revêtement formant barrière thermique comprend en outre :
une troisième couche (68) ayant une quatrième microstructure ; et une seconde intercouche (66) ayant une cinquième microstructure formée entre lesdites deuxième (64) et troisième (68) couches.

3. Article revêtu selon la revendication 2, dans lequel ladite quatrième microstructure a une microstructure sélectionnée à partir du groupe à colonnes, amorphe, aléatoire et semblable à une latte ;
et, de manière facultative, dans lequel ladite cinquième microstructure comprend une combinaison desdites deuxième et quatrième microstructures.

4. Article revêtu selon la revendication 1, dans lequel :
ledit article est un composant de moteur à turbine ;
ledit système de revêtement formant barrière thermique (38) dans lequel lesdites première et deuxième microstructures comprennent n'importe laquelle des microstructures suivantes : à colonnes, amorphe, aléatoire et semblable à une latte ; et
ladite troisième microstructure comprend une combinaison desdites première et deuxième microstructures.

5. Article revêtu selon la revendication 4, dans lequel chaque couche (40, 44 ; 60, 64, 68) dudit système de revêtement formant barrière thermique (38) comprend de la zircone stabilisée à l'oxyde d'yttrium ayant d'environ 1,0 % en poids à environ 25 % en poids d'oxyde d'yttrium du poids total de ladite couche et le reste de zircone ou de zircone stabilisée à l'oxyde de gadolinium ayant d'environ 5,0 % en poids à environ 99 % en poids d'oxyde de gadolinium du poids total de ladite couche et le reste de zircone ou à la fois de ladite zircone stabilisée à l'oxyde d'yttrium et de ladite zircone stabilisée à l'oxyde de gadolinium.

6. Article revêtu selon la revendication 5, dans lequel ladite zircone stabilisée à l'oxyde de gadolinium inclut d'environ 30 % en poids à environ 70 % en poids d'oxyde de gadolinium du poids total de ladite couche (40, 44 ; 60, 64, 68) et le reste de zircone.

7. Article revêtu selon la revendication 4, 5 ou 6, comprenant en outre une couche de revêtement de liaison (34 ; 54) disposée entre ladite au moins une surface et ledit système de revêtement formant barrière thermique (38) ;
et comprenant en outre de manière facultative une couche d'oxyde cultivée de façon thermique (36 ; 56) disposée entre ladite couche de revêtement de liaison (34 ; 54) et ledit système de revêtement formant barrière thermique (38).

8. Article revêtu selon l'une quelconque des revendications 4 à 7, dans lequel ledit revêtement formant barrière thermique comprend en outre :
une troisième couche (68) ayant une quatrième microstructure ; et
une seconde intercouche (66) ayant une cinquième microstructure formée entre lesdites deuxième (64) et troisième (68) couches,
dans lequel ladite quatrième microstructure comprend n'importe laquelle des microstructures suivantes : à colonnes, amorphe, aléatoire et semblable à une latte, et
dans lequel ladite cinquième microstructure comprend une combinaison desdites deuxième et quatrième microstructures.

9. Article revêtu selon l'une quelconque des revendications précédentes, dans lequel ladite conductibilité thermique est dans la plage de 2,0 à 16 BTU in/hr ft² F (0,29 à 2,31 W/mK).

10. Processus pour revêtir un article, comprenant :
l'application d'une première couche (40 ; 60) d'un système de revêtement formant barrière thermique (38) ayant une première microstructure à colonnes sur au moins une surface d'un article ;
l'application sur ladite première couche (40 ; 60) d'une deuxième couche (44 ; 64) dudit système de revêtement formant barrière thermique (38) ayant une deuxième microstructure sélectionnée à partir du groupe amorphe, aléatoire et semblable à une latte ; **caractérisé par**
la formation entre lesdites première (40 ; 60) et deuxième (44 ; 64) couches d'une intercouche (42 ; 62) ayant une troisième microstructure comprenant une combinaison desdites première et deuxième microstructures ; dans lesquelles
au moins une couche (40, 44 ; 60, 64, 68) dudit système de revêtement formant barrière thermique inclut :
une matière de base en céramique sélectionnée à partir du groupe constitué par un zirconate, un hafnate et un titanate ; et
au moins un oxyde d'un métal présent en une quantité d'environ 30 % en poids à environ 70 % en poids du poids total de ladite couche, ledit métal comprenant au moins un métal sélectionné à partir du groupe constitué par le lanthane, le cérium, le praséodyme, le néodyme, le prométhium, le samarium, l'europium, le gadolinium, le terbium, le dysprosium, l'holmium, l'erbium, le thulium, l'ytterbium, le lutécium, l'indium, le scandium et l'yttrium ; et
ledit système de revêtement formant barrière thermique (38) présente une conductibilité thermique non supérieure à 16 BTU in/hr ft² F (2,31 W/mK).

11. Processus selon la revendication 10, comprenant en outre les étapes suivantes :
application d'une couche de revêtement de liaison (34 ; 54) sur ladite au moins une surface dudit article avant d'appliquer ladite première couche (40 ; 60) ; et
formation d'une couche d'oxyde cultivée de façon thermique (36 ; 56) sur ladite couche de revêtement de liaison (34 ; 54) avant d'appliquer ladite première couche (40 ; 60) ; et
dans lequel, de manière facultative, lesdites étapes d'application de ladite première couche (40 ; 60), d'application de ladite deuxième couche (44 ; 64) et d'application de ladite couche de revêtement de liaison (34 ; 54) comprennent l'utilisation d'un processus de dépôt en phase vapeur ou d'un processus de pulvérisation thermique.
